

Sept. 23, 1969

F. L. WILLIAMS

3,468,988

METHOD OF FORMING CONCRETE STRUCTURES WITH TREATED FORM PANELS

Filed Jan. 21, 1965



INVENTOR  
FRANK L. WILLIAMS

BY *Dick Zerley*  
ATTORNEYS

3,468,988

## METHOD OF FORMING CONCRETE STRUCTURES WITH TREATED FORM PANELS

Frank L. Williams, Des Moines, Iowa, assignor, by mesne assignments, to International Concrete Systems Company, Bala Cynwyd, Pa., a corporation of Delaware  
Filed Jan. 21, 1965, Ser. No. 426,885  
Int. Cl. B28b 1/14, 7/36; E04b 1/16

U.S. Cl. 264—31

4 Claims

### ABSTRACT OF THE DISCLOSURE

A method for forming a concrete structure in an assembly of aluminum panels having inner surfaces defining a construction form in which the inner surface of the panels is treated with an oxidizing agent and an oil substance is subsequently applied to the treated surfaces. Concrete is then poured into the construction form to produce a formed structure. After hardening of the concrete, the panels are stripped from the formed structure.

This invention relates to a concrete wall construction panel and more particularly to a concrete wall construction panel having a film thereon which prevents the panel from sticking to concrete.

The use of concrete wall construction panels which are constructed of aluminum or aluminum alloys has become widespread in recent years. One disadvantage in aluminum construction panels is the tendency of them to stick to the concrete. This makes it rather difficult to remove the panels from the hardened concrete. Certain types of the aluminum construction panels cause a simulated brick effect to be formed in the finished concrete wall. The sticking of the construction panels to these surfaces result in the panels pulling off fragments of the hardened concrete when they are removed therefrom. This results in a somewhat less than desirable decorative surface on the concrete wall due to the holes, etc. caused by the fragments being pulled from the concrete.

Additionally, it has been found that the aluminum hydroxides in the concrete have a tendency to react with the aluminum forms thereby creating a serious problem for the builder.

Building contractors have attempted to prevent the construction panels from sticking to the concrete by oiling the interior faces of the construction panels. The use of oil on the construction panels has only been partially successful.

Therefore, it is a principal object of this invention to provide a concrete wall panel which has a film thereon to prevent it from sticking to the concrete.

A further object of this invention is to provide a concrete wall construction panel which will not react with the aluminum hydroxides in the concrete.

A further object of this invention is to provide a concrete wall construction panel which has a film formed integrally thereon which prevents the panel from sticking to concrete.

A further object of this invention is to provide a concrete wall construction panel which may be removed from a concrete wall without removing fragments of the wall.

A further object of this invention is to provide a concrete wall construction panel having a film thereon which does not come off the panel.

A further object of this invention is to provide a concrete wall construction panel having a film thereon which is formed by the reaction of the construction panel and the substance applied thereon.

It is a further object of this invention to provide a

concrete wall construction panel which is economical of manufacture, durable in use and refined in appearance.

These and other objects will be apparent to those skilled in the art.

This invention consists in the construction, arrangements, and combination of the various parts of the device, whereby the objects contemplated are attained as hereinafter more fully set forth, specifically pointed out in the claims, and illustrated in the accompanying drawings, in which:

10 FIG. 1 is a perspective view of the concrete wall construction panel;

FIG. 2 is a sectional view of the wall construction panel as seen on line 2—2 of FIG. 1 at an enlarged scale, and

15 FIG. 3 is a side sectional view illustrating the manner in which the concrete wall construction panels are utilized to form a concrete wall.

The numeral 10 generally designates the construction panel having an interior face 11 and exterior face 13 and edge flanges 15. As seen in FIG. 2, the numeral 17 represents a film which has been applied to the interior surface 11 of panel 10 to prevent the panel from sticking to the concrete which is generally indicated at 19 in FIG. 3.

20 Film 17 is formed on panel 10 by either of the following examples:

Example No. 1.—A quantity of caustic soda and a quantity of water are first heated. The heated caustic 30 soda-water solution is then applied to panel 10 by any convenient method such as by dipping panel 10 into the heated solution or by spraying the solution onto panel 10. It is only necessary to treat the inner surface of panels 10 as it is only the inner surface thereof which comes into contact with the concrete. Panel 10 is then allowed to dry. A soot colored film is formed on panel 10 due to the reaction of the aluminum and/or aluminum alloys in panel 10 with the caustic soda and water. This reaction causes film 17 to be bonded on panel 10 which prevents film 17 from being rubbed or washed therefrom.

35 While film 17 has never been chemically analyzed, it is believed that it is comprised of aluminum hydroxide or aluminum oxide. The resultant composition of film 17 would necessarily vary depending on the composition of panel 10.

40 It has been discovered that the most ideal proportion of caustic soda to water is approximately 5–10% by weight. While other proportions work with varying degrees of success, the foregoing range is the most desirable. It has also been found that the best results are obtained when the caustic soda-water solution is heated to 150–160 degrees Fahrenheit. Varying degrees of success are obtained in forming film 17 by varying the solution temperature but the foregoing range has been found to be the most desirable.

45 Example No. 2.—A quantity of muriatic acid is applied to panel 10 by any convenient means such as described in Example No. 1. The muriatic acid reacts with the aluminum and/or aluminum alloys in panel 10 to form 50 soot colored film thereon. The soot colored film of Example No. 2 is not quite as black as the soot colored film of Example No. 1. The reaction between panel 10 and the muriatic acid causes film 17 to be formed and to be bonded to panel 10 which aids in preventing film 17 from being rubbed or washed off panel 10. While the film 17 obtained in Example No. 2 has never been chemically analyzed, it is believed that film 17 is composed of aluminum chloride. The resultant composition of film 17 would necessarily vary depending on the composition of panel 10.

55 The normal method of operation is as follows: A plurality of panels 10, which have film 17 thereon, are as-

sembled to provide a wall construction form such as seen in FIG. 3. Panels 10 have also been coated with a layer or film of oil to further aid in removing the panels from the hardened concrete. The concrete is poured into the form and permitted to harden in conventional fashion. When the concrete has hardened, panels 10 are stripped or removed therefrom. Film 17 prevents panel 10 from reacting with the aluminum hydroxide and the concrete. Film 17 also prevents panel 10 from sticking to the concrete and insures that panel 10 may be removed from the hardened concrete without destroying the desired decorative effect thereon.

Thus from the foregoing it can be seen that the device accomplishes at least all of its stated objectives.

I claim:

1. A method for forming a concrete structure in an assembly of aluminum panels having inner aluminum surfaces defining a construction form comprising the steps of applying a sodium hydroxide solution to the inner surfaces of the panels, subsequently applying an oil substance to the surface treated with the sodium hydroxide solution, pouring concrete into the construction form defined by the inner surfaces, allowing the concrete to harden into a formed structure, and stripping the panels from the formed structure.

2. Method in accordance with claim 1 wherein sodium hydroxide is from 5% to 10% by weight of said solution.

3. Method in accordance with claim 1 wherein the solution applied to the inner surfaces of the panels is at a temperature of approximately 150° to 160° F.

5 4. A method for forming a concrete structure in an assembly of aluminum panels having inner aluminum surfaces defining a construction form comprising the steps of applying hydrochloric acid to the inner surfaces of the panels, subsequently applying an oil substance to the surfaces treated with the hydrochloric acid, pouring concrete into the construction form defined by the inner surfaces, allowing the concrete to harden into a formed structure, and stripping the panels from the formed structure.

10

#### References Cited

##### UNITED STATES PATENTS

|    |           |         |             |           |
|----|-----------|---------|-------------|-----------|
| 15 | 1,575,122 | 3/1926  | Madsen      | 117—5.3   |
|    | 2,669,752 | 2/1954  | Pratt       | 264—337 X |
|    | 2,806,277 | 9/1957  | Hand et al. | 264—34    |
|    | 3,217,356 | 11/1965 | Stursman    | 264—69 X  |

##### FOREIGN PATENTS

|    |         |         |                |
|----|---------|---------|----------------|
| 20 | 223,994 | 11/1924 | Great Britain. |
|    | 766,858 | 1/1957  | Great Britain. |

ROBERT F. WHITE, Primary Examiner

25 K. J. HOVET, Assistant Examiner

U.S. Cl. X.R.

106—38.22; 117—5.3; 249—115; 264—39, 338

30